

March 7, 1961

R. H. COMYN

2,974,029

NONGASEOUS PYROTECHNIC DELAY MIXTURE

Filed July 13, 1950



Inventor  
RAYMOND H. COMYN

By *L. D. O'Brien*  
*R. M. Hicks*

Attorneys

## 1

2,974,029

## NONGASEOUS PYROTECHNIC DELAY MIXTURE

Raymond H. Comyn, 316 Southampton Drive, Northwest Park Apts., Silver Spring, Md.

Filed July 13, 1950, Ser. No. 173,636

1 Claim. (Cl. 52—2)

(Granted under Title 35, U.S. Code (1952), sec. 266)

This invention relates to a nongaseous delay pyrotechnic mixture for use in a projectile, rocket, flare, smoke float, or any other ordnance missile or device and is particularly adapted to cause initiation of the explosive or propellant charge, light or smoke emitting pyrotechnic mixture, as the case may be, in time delayed relation with respect to the initial ignition thereof by the usual igniter associated therewith.

Heretofore, gaseous delay compositions used in ordnance missiles and devices by the armed forces for delaying the ignition of the pyrotechnic mixtures or explosives therein, such, for example, as a bursting charge, propellant charge, light or smoke emitting composition as the case may be, have not been altogether satisfactory for the reasons that such compositions were susceptible to changes in gas pressure and thus the burning range thereof was affected by the gas pressure produced therefrom during ignition and burning of such compositions thereby causing erratic burning rate thereof. Furthermore, such compositions lack stability, in that they would absorb sufficient moisture to reduce the efficiency and effect the burning rate thereof and upon numerous occasions fail to function altogether at low temperature particularly after being stored over a long period of time. Such compositions also proved not altogether satisfactory for the purpose intended inasmuch as the burning rate was erratic and unpredictable and the ignition sensitivity characteristic thereof was nonuniform.

The present invention is especially compounded to overcome the aforesaid objections found in prior art compositions and to provide a new and improved nongaseous delay mixture having the admirable characteristic of stability, sensitivity and uniform burning rate without noticeable gas evolution therefrom.

An object of this invention is to provide a new and improved nongaseous delay mixture for use in an ordnance missile which forms solid combustion products, and does not evolve an appreciable amount of gas during burning thereof.

Another object of the invention is to provide a stable nongaseous delay mixture having an ignition temperature lower than the burning temperature of the igniter associated therewith and which is ignited by the igniter whereupon the burning range of the mixture is unaffected by the gas pressure produced during the burning thereof.

Another object of the invention is to provide a sensitive nongaseous delay mixture whose burning rate is predictable, and which produces sufficient heat at a high temperature to ignite either a detonator or a relay igniter, as the case may be.

An additional object is to provide a method of producing a nongaseous pyrotechnic delay mixture.

Other objects and many of the attendant advantages of this invention will be readily appreciated as the same becomes better understood by reference to the following detailed description when considered in connection with the accompanying drawing wherein:

## 2

One adaptation of the invention is illustrated in the accompanying drawing which is a fragmentary longitudinal sectional view of an ordnance device.

The missile comprises the usual shell or casing 10 having a normally locked firing pin 11 adapted to be moved to a firing position in engagement with the primer 12 upon impact of the missile with a target, it being understood, however, that the firing pin is released for movement to the firing position when the detents 13 are moved out of engagement therewith by centrifugal force as the missile travels along a trajectory. Arranged within the cavity 14 formed in the shell 10 and having an igniter 15 on one end, and an igniter 16 on the other end thereof is the nongaseous delay mixture 17 of the present invention, the igniter 15 being adapted to be ignited by the primer 12 when the firing pin is moved to the firing position, whereupon the delay mixture is ignited by the igniter 15 and will burn at a predetermined rate, without noticeable gas evolution therefrom for a predetermined period of time such, for example, as from 3.83 to 4.05 seconds whereupon the igniter 16 is ignited by the delay mixture and thus the booster charge 18 is fired in time delayed relation with respect to impact of the missile with the target thereby firing the bursting charge 25 and exploding the missile.

The composition of the present invention possesses the characteristics which make it admirably suited for the uses indicated herein and comprises a mixture of cobalt as a metallic fuel, lead chromate and potassium perchlorate as a pair of oxidizing agents. The cobalt in powder form is treated first with a hot aqueous solution of potassium dichromate and then with a carbon tetrachloride solution of stearic acid prior to the mixing of the cobalt with the lead chromate and potassium perchlorate. This is done to protect the cobalt from deterioration.

A typical mixture producing satisfactory stability, sensitivity, burning rate and showing no appreciable gas evolution while burning is as follows:

|                       | Percent |
|-----------------------|---------|
| Cobalt                | 41      |
| Lead Chromate         | 47      |
| Potassium perchlorate | 12      |

It will be understood, however, that the proportions of these ingredients may be varied, if desired, to meet the requirements of various uses of the mixture.

The mixing of the ingredients may be accomplished in any suitable manner and during such mixing operation carbon tetrachloride may be added to reduce particle friction of the ingredients to a sufficiently low value to facilitate mixing.

Both wet and dry methods of mixing the ingredients have been tested and from such tests it has been found that while both methods are satisfactory the dry method of mixing in certain cases is most successful and has produced the best results. Furthermore, when the dry method is employed it does not require drying and regrinding after mixing as is the case when employing the aforesaid wet method. In preparing the ingredients comprising the nongaseous delay mixture of the instant invention it has been found that the most satisfactory results are obtained when the cobalt is of a particle size such, for example, as 100% less than the U.S. standard sieve, mesh size 325/000, the lead chromate is of such a particle size as to readily pass through a U.S. standard sieve, mesh size 200/000, and the potassium perchlorate of such a particle size as to pass through a U.S. standard sieve, mesh size 325/000. When the aforesaid preparation has been completed the ingredients are then thoroughly mixed in any suitable manner but preferably by placing them in a mixing device, the device being of

any type suitable for the purpose such, for example, as the type known in the trade as the "Simpson" mixer. During the mixing operation a quantity of carbon tetrachloride may be added to the ingredients, if desired, thereby reducing the friction between the particles thereof and also insure thorough mixing of the ingredients. The time period required to mix the aforesaid ingredients thoroughly when the mixer is set in operation is approximately 30 minutes, the ingredients being subjected to a mulling action as the mixer operates.

It has been found that ingredients comprising mixtures of this type may segregate during wet mixing with the lighter materials coming to the top, and it is probable that this condition may also occur during dry mixing of the ingredients and thus this effect can be minimized by employing chemicals as heretofore described, with densities and particle sizes which are approximately in the same range. Furthermore, it has been found that mixing is improved by employing as few chemicals as possible, such, for example, as disclosed in the instant invention, rather than four or five chemicals, as heretofore used in prior art devices.

It will be understood, however, that as either the metallic fuel or the oxidant in a mixture is increased over the amount necessary for maximum heat, the reaction heat measured in calories per gram, will decrease. Under some conditions an excess of metallic fuel may be undesirable; while an excess of oxidant may tend to decrease the burning rate of the mixture. However, a large excess of an oxidant may be undesirable if the oxidant releases its oxidizing element very easily.

The use of an inert diluent provides another method of reducing the reaction heat and the burning rate of the mixture. However, there is the possibility of actually stopping the whole reaction if the mixture is uneven. By the addition of a second oxidant, as heretofore described, which reacts with the fuel at a slower rate than the first oxidant thereby providing an effective method of slowing the burning rate of the mixture, and thus as long as the fuel and both of the oxidants are present in stoichiometric proportions, the danger of bubbles due to a sudden excess of oxygen being released by the oxidant is decreased whereupon uniform and complete burning of the mixture is insured.

It is well known in the art of delay mixtures that moisture accelerates the deterioration of gasless delay mixtures, such conditions resulting from the reaction of the ingredients of the mixture with moisture as well as from ionic reactions which are promoted by the solvent action of the moisture. In view of these conditions existing in prior art mixtures the instant invention overcomes such conditions by providing a mixture having the desirable characteristics of low water solubility; free from hydrate formation, and not subjected to decomposition in water.

The particle size of the oxidant does not affect the properties of a gasless delay element as much as the particle size of the fuel. As the particle size decreases and the surface thereof increases, acceleration of the burning rate of the gasless delay element and surveillance deterioration thereof may be expected. However,

it is desirable to use a fuel whose particle size lies in the subsieve range for the reason that they ignite more readily as the size decreases.

During tests, the gasless delay mixture and the starter 5 and relay igniter compositions therefor were loaded in a steel test body at pressures from 10,000 to 35,000 p.s.i., the delay element being composed of three equal increments and disposed between the aforesaid igniters. The exposed top portion of the starter composition was 10 ignited by any convenient means, whereupon the delay element proved to be sufficiently sensitive to be ignited by the starter igniter, the time required for the delay element to burn to the bottom was substantially 4.05 seconds, the burning temperature thereof being sufficiently high to cause ignition of the relay igniter. Furthermore, the test proved that the gasless delay mixture burned evenly and at a relatively slow rate when ignited, without noticeable gas evolution therefrom.

In loading the gasless delay mixture into the delay 20 cavity of an ordnance missile or device it has been found that the best results were obtained when the aforesaid increments were pressed into the cavity at a pressure of 10,000 to 35,000 p.s.i.

From the foregoing, it will be understood, that a gas- 25 less delay mixture for an ordnance missile or device has been compounded either by wet or dry mixing methods disclosed herein and having new and improved characteristics such, for example, as uniform mixing and surveillance qualities; whose burning range is un- 30 affected by the gas pressure produced during burning thereby permitting the delay mixture to burn evenly until entirely consumed; and which is sufficiently sensitive to be ignited by the starter igniter and to furnish sufficient heat at a high enough temperature to ignite either 35 a relay igniter or a detonator, as the case may be, and which will not evolve an appreciable amount of gas during burning thereof.

Obviously many modifications and variations of the 40 present invention are possible in the light of the above teachings. It is therefore to be understood that within the scope of the appended claims the invention may be practiced otherwise than as specifically described.

The invention described herein may be manufactured 45 and used by or for the Government of the United States of America for governmental purposes without the payment of any royalties thereon or therefor.

What is claimed as new and desired to be secured by Letters Patent of the United States is:

The method of producing a nongaseous pyrotechnic 50 delay mixture which comprises the steps of first treating a quantity of powdered cobalt with a hot aqueous solution of potassium dichromate and thereafter treating the cobalt with a carbon tetrachloride solution of stearic acid, and mixing the treated cobalt with quantities of 55 lead chromate and potassium perchlorate.

#### References Cited in the file of this patent

#### UNITED STATES PATENTS

- |    |           |                |              |
|----|-----------|----------------|--------------|
| 60 | 1,308,342 | Du Pont        | July 1, 1919 |
|    | 2,457,860 | Bennett et al. | Jan. 4, 1949 |